

# UNITED STATES PATENT OFFICE.

JOHN FARREL, OF NEW YORK, N. Y.

## METALLIC ALLOY FOR SAFES.

SPECIFICATION forming part of Letters Patent No. 298,365, dated May 13, 1884.

Application filed November 2, 1883. (Specimens.)

*To all whom it may concern:*

Be it known that I, JOHN FARREL, of New York city, New York, have invented a Metallic Alloy for Safes, whereof the following is 5 a specification.

The metal made from franklinite ore is one of the hardest metals known, and, being well adapted for resisting the action of drills and other cutting-tools, is extensively used by myself and others in the construction of burglar-proof safes. It is, however, more or less porous and friable from the peculiarity of its crystalline structure, and this friability is a weakness, inducing the metal to pulverize under the drill when applied with great pressure. My new alloy is not thus susceptible, and yet is as hard as or harder than franklinite and metals of the same character. It is made by melting up tin-scrap—such as the waste or scraps from tinware-manufacture—and combining the same with soft wrought-iron, combined with the franklinite iron, or that made from the spathic ores. It may be variously made; but I have practiced the following way 20 with success: I take the tin-plate scraps, melt them down, and run the metal into molds for castings of a convenient form for remelting. I then take about an equal quantity, by weight, of this compound and of a franklinite iron, 25 put both in a cupola, and fuse them together at a very high heat. I then draw off this molten metal and pour it into molds prepared and adapted for bringing out the article or articles desired. Another way is to compress 30 the scrap-tin into bundles and melt it up with the franklinite at once. The metal or alloy so compounded when cold is harder, tougher,

and more dense and compact than franklinite alone, and as a drill resistant is superior to any metal or alloy hitherto known. It is 40 therefore specially adapted for the walls of burglar-proof safes, and because its hardness is natural and cannot be affected by the local application of heat. The alloy may also be used for journal-boxes, for dies for stamping, 45 and rolls for rolling sheet metals, and for other purposes. All articles made from this metal or alloy should be cast at once to the size and shape required, if possible; and if not, the finishing must be by grinding the surface—as by 50 corundum-wheels—because it is nearly impossible to work the metal with cutting-tools.

My said invention is restricted to the ingredients herein specified. Nevertheless, I do not confine myself to the exact proportions 55 indicated, but shall vary the same when found necessary; and instead of the franklinite the similar metal known as "spiegeleisen" may be substituted with good effect; but the franklinite is preferable. 60

I claim as my invention—

1. The new composite metal or alloy of tin-plate scrap, iron, and franklinite iron or its equivalent, substantially as described.
2. The method of forming a composite metal 65 of tin-plate scrap, iron, and franklinite iron or its equivalent, substantially as described, consisting in melting the ordinary tin-scrap to form an alloy, and fusing this alloy at the same time or subsequently with the franklinite.

JOHN FARREL.

Witnesses:

EARLE H. SMITH,  
W. D. VAN RODE.